

1

3,377,148

### GASOLINE FUEL COMPOSITION

Richard J. DeGray, South Euclid, and John S. Mann, Warrensville Heights, Ohio, assignors to The Standard Oil Company, Cleveland, Ohio, a corporation of Ohio  
No Drawing. Filed Mar. 15, 1965, Ser. No. 439,993  
7 Claims. (Cl. 44—63)

The present invention relates to an improved gasoline and to the method of its manufacture and more particularly pertains to a high octane gasoline containing tetraalkyl lead and a reaction product of an amide and a monocarboxylic acid or its anhydride or acid halide as lead appreciator and to the process for manufacture thereof.

The present invention deals with a novel class of gasoline additives which increase the octane number of leaded motor fuels. These additives, or "tetraalkyl lead extenders" as they are sometimes referred to, consist of gasoline soluble reaction products of a monocarboxylic acid or its anhydride with an amide having the grouping



The additives most useful in the present invention include the following:



wherein R is a hydrocarbon group having from 1 to 18 carbon atoms, R<sup>1</sup> and R<sup>2</sup> are hydrogen or an alkyl group having from 1 to 4 carbon atoms, R<sup>3</sup> is a hydrocarbon group having from 1 to 6 carbon atoms, R<sup>4</sup> is a hydrocarbon group having from 1 to 18 carbon atoms, R<sup>5</sup> is a hydrocarbon diradical having from 1 to 12 carbon atoms, R<sup>6</sup> is hydrogen or a hydrocarbon group having from 1 to 12 carbon atoms and R<sup>7</sup> is a hydrocarbon diradical having from 1 to 12 carbon atoms. More preferred in the present invention are compounds of the foregoing types wherein R is an alkyl group having from 1 to 18 carbon atoms, R<sup>1</sup> and R<sup>2</sup> are each independently hydrogen or an alkyl group containing from 1 to 4 carbon atoms, R<sup>3</sup> is an alkyl or alkenyl group having from 1 to 6 carbon atoms, R<sup>4</sup> is an alkyl or alkenyl group containing from 1 to 18 carbon atoms, R<sup>5</sup> is an alkylene group having from 1 to 6 carbon atoms, R<sup>6</sup> is an alkyl group having from 1 to 12 carbon atoms and R<sup>7</sup> is an alkenylene group having from 1 to 12 carbon atoms. Specific compounds of the foregoing types which are particularly preferred in the present invention include:

2



In the foregoing compounds the exact structure of the acid adducts with the various amides is unknown. The acid adducts are prepared by mixing the carboxylic acid and the amide. The acetylated amides are prepared by reacting the amide which contains at least one hydrogen bonded to the amide nitrogen with the carboxylic acid anhydride or acyl halide.

The effective concentration of the additives of this invention in leaded motor fuel range from about 0.05 to about 3% by weight based on the weight of the motor fuel, with maximum benefits being derived in the range of from about 0.5 to 1.5% by weight of the additive.

The increase in octane number obtained with the additives of this invention in a given gasoline varies with the concentration of the additive, the concentration of tetraethyl lead in the gasoline as well as the type of fuel employed. Maximum response to the additives is obtained in an aromatic fuel. The additives also are generally more effective with increased concentration of the tetraalkyl lead in the gasoline. The amount of tetraalkyl lead in the gasolines useful in the present invention can vary from 1 to 6 ml. of tetraalkyl lead per gallon of gasoline.

The acid adduct additives of this invention may be prepared at moderate temperatures, i.e., at room temperature or slightly above, by simply mixing the amide with the acid. The reactants are generally miscible and normally a solvent is not necessary for carrying out the reaction. If desired, the reaction may be carried out in the presence of a solvent such as toluene or a catalytically reformed hydrocarbon, particularly in instances in which one of the reactants is a solid. Generally the formation of the carboxylic acid-amide adduct is exothermic.

As was indicated earlier, the exact nature of the carboxylic acid-amide adducts is not known but they are probably combined by primary or secondary chemical bonding or by a combination of these two types of bonds.

The reaction product of amides containing at least one hydrogen on the amide nitrogen with carboxylic acid or acyl halides are believed to be acylated amides.

This invention is further illustrated in the following example.

### EXAMPLE

The additives used were prepared as follows:

(A) N-dodecyl trimethylene urea-acetic acid adduct,



was prepared by heating and stirring in a 500 ml. reactor flask fitted with a stirrer and condenser a mixture of 58.8 g. of n-dodecyl amine, 11.2 g. of urea and approximately 100 ml. of toluene. The reaction was carried out under reflux and ammonia was evolved from the top of the condenser. After about two hours the reaction had been completed. The reaction mixture was then cooled to room temperature and to it were added 11.2 g. of glacial acetic acid. Upon shaking the mixture there was a definite evolution of heat. Similar results were obtained when the foregoing reaction was carried out in the absence of toluene.

(B) Pyrrolidone-acetic acid adduct was prepared by mixing 17.02 g. of pyrrolidone and 12.01 g. of glacial acetic acid at a temperature slightly above 25° C. (the melting point of pyrrolidone). The heat of reaction increased the temperature of the mixture and the resulting solution was a homogeneous liquid.

(C) Pyrrolidone-acetic acid adduct was prepared as in B except that 18.72 g. of pyrrolidone were reacted with 12.01 g. of acetic acid.

(D) N-methyl pyrrolidone-acetic acid adduct was prepared by mixing 19.82 g. of N-methyl pyrrolidone and 12.01 g. of glacial acetic acid with stirring at about room temperature. Heat was evolved from the reaction and the final solution was a homogeneous product.

(E) N-methyl pyrrolidone-acetic acid adduct was prepared as in D except that 20.80 g. of N-methyl pyrrolidone were reacted with 12.01 g. of glacial acetic acid.

(F) N-oleyl trimethylene urea-acetic acid adduct was prepared by a procedure similar to that given in A using 80.4 g. of oleyl amine and 12.01 g. of urea. To this reaction mixture were added 12.01 g. of acetic acid.

(G) Acetylated pyrrolidone was prepared by mixing 34.04 g. of pyrrolidone and 20.42 g. of acetic anhydride in a 250 ml. flask. The mixture was heated to 110° C. and this was accompanied by a gradual change in color of the reaction mixture to a dark brown color. At 160° C. the reaction appeared to be complete. The product was homogeneous and soluble in gasoline.

(H) Pyrrolidone-acrylic acid adduct was prepared by mixing 85.10 g. of pyrrolidone and 72.06 g. of acrylic acid with stirring. A considerable amount of heat was evolved. The product was a homogeneous liquid at room temperature.

5 The properties of the fuels (1-3) used are as follows:

| Properties of Fuel 1 |                                   | ASTM D-86 |      |
|----------------------|-----------------------------------|-----------|------|
|                      |                                   | Percent   | ° F. |
| 30                   | Percent Saturates, 53             | 10        | 144  |
|                      | Percent Olefins, 6                | 30        | 205  |
|                      | Percent Aromatics, 41             | 50        | 243  |
|                      | Reid Vapor Pressure, p.s.i., 7.69 | 70        | 275  |
|                      | Gravity at 60° F., 0.7636         | 90        | 337  |
|                      | Tetraethyl Lead, cc./gal., 2.39   | (1)       | 405  |

| Properties of Fuel 2               |     | ASTM D-86 (Distillation Test) |      |
|------------------------------------|-----|-------------------------------|------|
|                                    |     | Percent                       | ° F. |
| Percent Saturates, 70.             | 10  | 141                           |      |
| Percent Olefins, 8.                | 30  | 202                           |      |
| Percent Aromatics, 23.             | 50  | 238                           |      |
| Reid Vapor Pressure, p.s.i., 0.91. | 70  | 275                           |      |
| Gravity at 60° F., 0.7388.         | 90  | 344                           |      |
| Tetraethyl Lead, cc./gal., 2.58.   | (1) | 394                           |      |

| Properties of Fuel 3              |         | ASTM D-86 |
|-----------------------------------|---------|-----------|
|                                   | Percent | ° F       |
| Percent Saturates, 40             | 10      | 163       |
| Percent Olefins, 17               | 30      | 218       |
| Percent Aromatics, 43             | 40      | 258       |
| Reid Vapor Pressure, p.s.i., 4.39 | 70      | 306       |
| Gravity at 60° F., 0.7872         | 90      | 366       |
| Tetraethyl Lead, cc./gal., 3.05   | (1)     | 433       |

---

### 1 End Point.

55 Engine data illustrating the lead appreciator response obtained using the standard F-1 and F-2 octane test procedures are shown in Tables I, II, III and IV. The additive compositions, additive concentrations and tetraethyl lead concentrations were varied and the results were compared 60 with tertiary butyl acetate at its most effective concentration.

TABLE I—E-1 OCTANE RESPONSE

| Lead Level, cc./gal.   | 0    |      |      | 1.5  |      |      | 3.0  |      |      |
|------------------------|------|------|------|------|------|------|------|------|------|
| Additive               | B    | H    | G    | B    | H    | G    | B    | H    | G    |
| Concentration:         |      |      |      |      |      |      |      |      |      |
| Blank                  | 98.1 |      |      | 97.1 |      |      | 98.7 | 98.9 | 98.7 |
| 0.25%                  |      |      |      |      |      |      | +1.0 | +0.7 | +1.5 |
| 0.50%                  |      |      |      |      |      |      | +1.5 | +1.1 | +1.0 |
| 0.75%                  | +0.1 | +0.1 | +0.1 | +0.7 | +0.6 | +1.1 | +2.4 | +1.5 | +1.4 |
| 1.00%                  |      |      |      |      |      |      | +2.0 | +1.4 | +1.7 |
| 1.25%                  | +0.2 | +0.3 | +0.3 | 0    | -0.2 | +0.7 | +1.4 | +1.0 | +2.0 |
| 1.50%                  |      |      |      |      |      |      | +1.3 | +0.8 | +2.2 |
| 1.75%                  | +0.6 | +0.4 | +0.6 | -0.3 | -0.7 | +0.6 | +0.8 | +0.4 | +1.7 |
| 0.750% + Butyl Acetate |      | +0.1 |      |      | +0.5 |      | +0.8 | +0.6 | +0.9 |

27.1. N. 2

TABLE II.—F-2 OCTANE RESPONSE

| Lead Level, cc./gal.  | 0    |      |      | 1.5  |      |      | 3.0  |      |      |
|-----------------------|------|------|------|------|------|------|------|------|------|
|                       | B    | H    | G    | B    | H    | G    | B    | H    | G    |
| Concentration:        |      |      |      |      |      |      |      |      |      |
| Blank                 | 81.1 |      |      | 86.8 |      |      | 87.3 | 87.8 | 87.5 |
| 0.25%                 |      |      |      |      |      |      | +1.0 | +0.7 | +1.0 |
| 0.50%                 |      |      |      |      |      |      | +1.6 | +1.2 | +0.8 |
| 0.75%                 | 0    | +0.1 | +0.1 | +0.2 | 0    | +0.6 | +1.9 | +1.7 | +1.8 |
| 1.00%                 |      |      |      |      |      |      | +1.7 | +1.8 | +1.7 |
| 1.25%                 | +0.5 | +0.4 | +0.2 | -0.2 | -0.6 | +0.4 | +1.8 | +1.2 | +1.8 |
| 1.50%                 |      |      |      |      |      |      | +1.1 | +0.8 | +1.7 |
| 1.75%                 | +0.5 | +0.5 | +0.6 | -0.3 | -0.6 | -0.1 | +1.0 | +0.6 | +1.8 |
| 0.75% t-Butyl Acetate |      | -0.2 |      |      | +0.1 |      | +1.3 | +1.0 | +1.2 |

Fuel: No. 3.

At the 3 cc. lead level, the additives of this invention exhibit their most favorable response, which in some cases is double the increase afforded by tertiary butyl acetate.

The optimum concentration for the reaction products of pyrrolidone with acetic acid and acrylic acid was found in the region of 0.5 to 1.5 weight percent. With the N-acetyl pyrrolidone, however, a peak in the response curve appeared at about 0.25% concentration at the 3 cc. tetraethyl lead level.

The effect on octane number of reaction products of acetic acid with acetamide and the product



wherein R is an alkyl group having from 8 to 10 carbon atoms, and R<sup>1</sup> and R<sup>2</sup> are methyl groups are shown in Table III. These data indicate that considerable increase in octane number in both the F-1 and F-2 ratings is obtained with these additives.

TABLE III

|                                                                                                                                                                 | F-1<br>Octane<br>Number | F-2<br>Octane<br>Number |
|-----------------------------------------------------------------------------------------------------------------------------------------------------------------|-------------------------|-------------------------|
| Blank (Fuel No. 3 plus 3 cc. tetraethyl lead)                                                                                                                   | 93.4                    | 87.2                    |
| 0.75% Dimethyl Acetamide-Acetic Acid                                                                                                                            | 100.3                   | 89.8                    |
| $\begin{array}{c} \text{O} \quad \text{CH}_3 \\ \parallel \\ \text{C}_8\text{H}_{17}-\text{C}-\text{N}(\text{CH}_3)\text{COOH} \\   \\ \text{CH}_3 \end{array}$ | 99.3                    | 88.8                    |

The octane response of the reaction products of N-oleyl and N-dodecyl derivatives of trimethylene urea with acetic acid are shown in Table IV.

TABLE IV.—OCTANE RESULTS

| Fuel Treatments                                          | F-1              |                    | F-2              |                    |
|----------------------------------------------------------|------------------|--------------------|------------------|--------------------|
|                                                          | Octane<br>Number | Δ Octane<br>Number | Octane<br>Number | Δ Octane<br>Number |
| Blank (Fuel No. 1 plus 3.5 cc. Tetraethyl Lead per gal.) | 101.1            |                    | 92.5             |                    |
| 1.00% Additive A                                         | 101.7            | +0.6               | 92.4             | -0.1               |
| Blank (Fuel No. 1 plus 3.2 cc. Tetraethyl Lead per gal.) | 101.4            |                    | 92.7             |                    |
| 0.5% Additive F                                          | 101.8            | +0.4               | 92.8             | +0.1               |
| 1.0% Additive F                                          | 102.0            | +0.6               | 93.1             | +0.4               |

The effect of N-methyl pyrrolidone-acetic acid adduct and related compounds are disclosed in Table V. It is interesting to note that pyrrolidone itself at 1% by weight concentration shows a significant increase of 0.4 octane, but the effect is not as great as that shown by the acetic acid reaction product with pyrrolidone. The addition of excess pyrrolidone to the acetic acid reaction product of pyrrolidone results in no additional increase in octane number.

TABLE V.—OCTANE DATA

| Fuel Treatments  | F-1              |                    | 70 |
|------------------|------------------|--------------------|----|
|                  | Octane<br>Number | Δ Octane<br>Number |    |
| Blank            | 100.8            |                    |    |
| 1.0% Additive B  | 101.5            | +0.7               |    |
| 1.0% Additive C  | 101.5            | +0.7               |    |
| 1.0% Pyrrolidone | 101.2            | +0.4               |    |
| 1.0% Additive D  | 101.4            | +0.6               |    |
| 1.0% Additive E  | 101.3            | +0.5               |    |

We claim:

1. A gasoline containing from 1 to 6 ml. of tetraalkyl lead per gallon and from 0.05 to 3% by weight of a lead appreciator selected from the group consisting of:



and



5

wherein R is a hydrocarbon group having from 1 to 18 carbon atoms, R<sup>1</sup> and R<sup>2</sup> are members selected from the group consisting of hydrogen and an alkyl group having from 1 to 4 carbon atoms, R<sup>3</sup> is a hydrocarbon group having from 1 to 6 carbon atoms, R<sup>4</sup> is a hydrocarbon group having from 1 to 18 carbon atoms, R<sup>5</sup> is a hydrocarbon group having from 1 to 12 carbon atoms, R<sup>6</sup> is a member from the group consisting of hydrogen and a hydrocarbon group having from 1 to 12 carbon atoms and R<sup>7</sup> is a hydrocarbon diradical having from 1 to 12 carbon atoms.

2. The gasoline of claim 1 wherein the lead appreciator is



10

3. The gasoline of claim 1 wherein the lead appreciator is



25

4. The gasoline of claim 1 wherein the lead appreciator is



30

2,324,118 7/1943 Sweeney ----- 44-72  
2,978,303 4/1961 Becker ----- 44-63  
2,991,162 7/1961 Malec ----- 44-63

35

FOREIGN PATENTS  
230,132 9/1960 Australia.

DANIEL E. WYMAN, Primary Examiner.

40 Y. H. SMITH, Assistant Examiner.

5. The gasoline of claim 1 wherein the lead appreciator is



10

6. The gasoline of claim 1 wherein the lead appreciator is



20

7. The gasoline of claim 1 wherein the lead appreciator is



25

#### References Cited

##### UNITED STATES PATENTS

2,324,118 7/1943 Sweeney ----- 44-72  
2,978,303 4/1961 Becker ----- 44-63  
2,991,162 7/1961 Malec ----- 44-63

30

FOREIGN PATENTS  
230,132 9/1960 Australia.

DANIEL E. WYMAN, Primary Examiner.

Y. H. SMITH, Assistant Examiner.